

## UNITED STATES PATENT OFFICE

1,947,038

COLORATION OF MATERIALS MADE WITH  
OR CONTAINING CELLULOSE ACETATE

George Holland Ellis and Henry Charles Olpin,  
Spondon, near Derby, England, assignors to  
Celanese Corporation of America, a corpora-  
tion of Delaware

No Drawing. Application October 8, 1928, Serial  
No. 311,252, and in Great Britain November 7,  
1927

3 Claims. (Cl. 8—5)

This invention relates to the dyeing, printing or stencilling of filaments, threads, yarns, fabrics, films or other products made with or containing cellulose acetate.

5 Prior U. S. Patent No. 1,618,415 describes the dyeing or otherwise coloring of cellulose acetate materials with unsulphonated nitro derivatives of diarylamines.

10 As the result of further research we have dis-  
covered that particularly fast and therefore very  
valuable dyeings, printings and stencillings may  
be obtained by means of compounds having the  
formula

15



where R represents a benzene ring substituted by  
20 alkyl, alkoxy or acetyl amino, and X represents  
a halogen atom.

As examples of the bodies which may be ap-  
plied according to the present invention the fol-  
lowing may be mentioned:—para-tolyl-4-chlor-  
25 2-nitraniline; meta-tolyl-4-chlor-2-nitraniline;  
4'-ethoxy-phenyl - 4 - chlor - 2 - nitraniline; 4'-  
methoxy-phenyl-4-brom-2-nitraniline; 4'-acetyl-  
amino-phenyl-4-chlor-2-nitraniline.

These bodies are all new compounds and may  
30 be obtained by condensation of the appropriate  
amino compound with the appropriate nitro-  
dihalogen-benzene. They may be applied to the  
goods by any suitable method, for example in  
35 aqueous solution, suspension or dispersion. Sus-  
pensions or dispersions thereof may be obtained  
for instance by fine grinding and suspending in  
aqueous baths or pastes, which may or may not  
be made acid or alkaline and to which protective  
40 colloids such as glue, starch, gums or the like  
may be added if desirable; by first dissolving in  
an organic solvent and pouring into water con-  
taining or not containing a protective colloid, or  
by pretreating the bodies with suitable dispersing  
45 agents. Such dispersing agents are for instance  
those of prior U. S. Patents 1,618,413 and 1,618,414  
granted February 22, 1927, 1,694,413 granted De-  
cember 11, 1928 and 1,716,721 granted June 11,  
1929 and a British Patent 273,819, viz. bodies of  
50 oily or fatty characteristics, namely higher fatty  
acids or sulphonated or other derivatives thereof  
containing salt-forming groups, such as sul-  
phoricinoleic acid or other sulphonated fatty  
acids or salts of such acids or bodies, for in-  
stance their alkali or ammonium salts, used alone  
55 or in conjunction with auxiliary solvents as de-

scribed in U. S. Patent No. 1,690,481 granted  
November 6, 1928 and British Patent No. 269,960;  
carbo-cyclic compounds containing in their  
structure one or more salt-forming groups or  
salts of such compounds; sulpho-aromatic fatty  
60 acids, such as sulpho-benzene stearic acid, sul-  
pho-phenol stearic acid, sulpho-naphthalene  
stearic acid or sulpho-naphthalene ricinoleic  
acid, or salts thereof; and soluble resin soaps or  
sodium or other soluble salts or soaps of resin  
65 acids.

The nitro bodies of the present invention may  
be employed not only for the dyeing, printing  
and stencilling of goods consisting wholly of  
70 cellulose acetate but also for the dyeing, print-  
ing and stencilling of mixed yarns, fabrics or  
materials containing, in addition to cellulose  
acetate, other materials such as cotton or other  
natural or artificial cellulose fibres, wool, silk  
75 and so forth. In general the bodies do not dye  
cotton and only slightly tint silk and wool. Thus  
mixed goods can be dyed, printed or stencilled  
to show differential or solid effects as desired,  
appropriate dyes or coloring matters being ap-  
80 plied if required to the non-acetate portion of the  
mixed material, either separately or simultane-  
ously with the nitro bodies of the present inven-  
tion.

The following examples illustrate the invention  
85 but are not to be considered as limiting it in  
any way:—

## Example 1

To dye a golden yellow shade on 10 kilos of cel-  
lulose acetate knitted fabric:—

100 grams of the dyestuff para-tolyl-4-chlor-2-  
nitraniline are ground to a fine powder and added  
to 500 grams of neutral sodium sulpho-ricino-  
leate (50%). The whole is heated to 95-100° C.  
95 till a good dispersion is obtained, and then diluted  
with boiling water, and added through a filter  
cloth to a dyebath containing 300 litres of soft  
water. The goods are entered and the tempera-  
ture raised during 3/4 hour to 75-80° C. and main-  
tained at this temperature till the desired shade  
is achieved. The fabric is then lifted, rinsed, and  
dried or otherwise treated as requisite. The shade  
is of exceptionally good fastness to light.

## Example 2

105 To dye 25 kilos of fabric composed of cotton  
and acetyl cellulose yarns in equal proportions  
so that a green shade is obtained on the cotton  
and a golden orange shade on the acetyl cellulose,

the cotton is first dyed in a suitable machine, the dyebath being prepared as follows:—

- 600 litres of soft water are heated to 30° C. and 12 litres of a 32.5% solution of sodium para-cresolate added. Into this is sieved 2.5 kilos of the anthraquinonoid vat dyestuff obtained by oxidation of dibenzanthrone and subsequent treatment with methyl sulphate and known as Caledon jade green paste (Color Index No. 1101). 750 grams of sodium hydrosulphite powder are now dredged in and the bath raked over gently until reduction is complete. The previously scoured-off material is entered and worked 20 minutes during which time the temperature is raised to 50° C. dyeing being continued at this temperature for a further 15 minutes when the goods are removed from the bath, squeezed, oxidized in air or in a bath containing 1 gram per litre of olive oil soap and 1 gram per litre of sodium perborate at 75° C.
- 20 The acetyl cellulose component is now dyed a golden orange shade as follows:—
- 25 250 grams of ground 4-ethoxy-phenyl-4-chlor-2-nitraniline are well stirred or ground with 2.5 litres of sodium-ricinoleate (50%). The mixture is heated under an open steam pipe and then diluted with boiling water and further boiled. The liquor is then filtered into a dye-bath containing cold soft water. The material is introduced and dyeing carried out while raising the temperature from 60 to 75° C., the volume of the bath being about 30:1 on the weight of the material.

In the appended claims the term dyeing is to be understood to include printing and stencilling.

What we claim and desire to secure by Letters Patent is:—

1. Process for dyeing materials comprising cellulose acetate comprising applying thereto a body having the formula



85

where R is a benzene ring containing an alkyl group or an acetyl amino group and X is a halogen.

2. Process for dyeing materials comprising cellulose acetate comprising applying thereto a body having the formula



95

where R is a benzene ring containing in the para position an alkyl group or an acetyl-amino group and X is a halogen.

3. Process for dyeing materials comprising cellulose acetate comprising applying thereto para-tolyl-4-chlor-2-nitraniline.

GEORGE HOLLAND ELLIS.  
HENRY CHARLES OLPIN.

105

110

45

40

115

45

120

50

125

55

130

60

135

65

140

70

145

75

150